

# United States Patent [19]

Shaw

[11] 3,898,109

[45] Aug. 5, 1975

[54] **HEAT TREATMENT OF  
NICKEL-CHROMIUM-COBALT BASE  
ALLOYS**

[75] Inventor: **Stuart Walter Ker Shaw, Wylde  
Green, England**

[73] Assignee: **The International Nickel Company,  
Inc., New York, N.Y.**

[22] Filed: **Jan. 2, 1974**

[21] Appl. No.: **430,111**

[30] **Foreign Application Priority Data**

Sept. 6, 1973 United Kingdom..... 41888/73

[52] **U.S. Cl.** ..... **148/162; 75/134 F; 75/171;**  
148/13; 148/32.5

[51] **Int. Cl.** ..... **C22c 19/00; C22f 1/10**

[58] **Field of Search** ..... **75/134 F, 171; 148/13,  
148/32, 32.5, 162**

[56] **References Cited**

UNITED STATES PATENTS

|           |         |                        |         |
|-----------|---------|------------------------|---------|
| 2,766,155 | 10/1956 | Betteridge et al. .... | 148/162 |
| 3,356,542 | 12/1967 | Smith.....             | 148/162 |
| 3,459,545 | 8/1969  | Bieber et al. ....     | 75/171  |

|           |         |                      |         |
|-----------|---------|----------------------|---------|
| 3,479,157 | 11/1969 | Richards et al. .... | 75/171  |
| 3,536,542 | 10/1970 | Murphy et al. ....   | 148/162 |
| 3,653,987 | 4/1972  | Boesch.....          | 148/162 |
| 3,667,938 | 6/1972  | Boesch.....          | 148/162 |
| 3,723,107 | 3/1973  | Richards.....        | 148/162 |
| 3,741,821 | 6/1973  | Athey et al. ....    | 148/162 |
| 3,748,192 | 7/1973  | Boesch.....          | 148/162 |

**FOREIGN PATENTS OR APPLICATIONS**

|           |         |                     |        |
|-----------|---------|---------------------|--------|
| 731,441   | 6/1955  | United Kingdom..... | 75/162 |
| 715,140   | 9/1954  | United Kingdom..... | 75/162 |
| 777,703   | 6/1957  | United Kingdom..... | 75/162 |
| 1,053,109 | 12/1966 | United Kingdom..... | 75/162 |
| 1,196,714 | 7/1970  | United Kingdom..... | 75/162 |
| 1,333,354 | 10/1973 | United Kingdom..... | 75/162 |

*Primary Examiner*—C. Lovell

*Attorney, Agent, or Firm*—Raymond J. Kenny; Ewan C. MacQueen

[57]

**ABSTRACT**

A four-stage heat-treatment to improve the stress-rupture life and stress-rupture ductility at elevated temperatures of nickel-chromium alloys in which a two-stage heat-treatment is used intermediate of an initial solution treatment and a final aging treatment.

**8 Claims, No Drawings**

HEAT TREATMENT OF  
NICKEL-CHROMIUM-COBALT BASE ALLOYS

The instant invention relates to the heat-treatment of nickel-chromium-cobalt base high-temperature alloys.

In my United States application No. 241,443, now abandoned, there is described and claimed castable nickel-chromium-cobalt alloys containing about 0.02 to 0.25 percent carbon, about 20 to 25 percent chromium, about 5 to 25 percent cobalt, one or both of molybdenum up to 3.5 percent and tungsten up to 5 percent in such amounts that the value 0.5 percent Mo) plus %W is from 0.5 to 5 percent, about 1.5 to 5 percent titanium and 1 to 5 percent aluminium, with the provisos that the sum of the aluminium and titanium (i) be from 4 to 7 percent and (ii) in tungsten-free alloys not exceed 6 percent, and further that the (iii) ratio of titanium to aluminium be from 0.75:1 to 4:1, about 0.5 to 3 percent tantalum, up to 3 percent niobium, about 0.005 to 1 percent zirconium and up to 2 percent hafnium, with the proviso that the value of percent Zr + 0.5 (percent Hf) be from 0.01 to 1 percent, about 0.001 to 0.05 percent boron, and up to 0.2 percent in total of yttrium or lanthanum or both, the balance, apart from impurities, being nickel in an amount of at least 30 percent.

In order to develop a high level of stress-rupture strength at elevated temperatures such as 927°C (1700°F) or 980°C (1,800°F), the alloys were to be subjected, upon casting, to a heat-treatment comprised of solution-heating and subsequent aging. Various heat-treatments of this general kind were given in my said U.S. Application, namely:

- a. Solution-heating at 1,050°-1250°C for 1-10 hours; aging at 600°-950°C for 1-24 hours.
- b. Solution-heating at 1,050°-1,250°C for 1-20 hours; intermediate heating at 800°-1,150°C for 1-16 hours; aging at 600°-950°C for 1-24 hours.
- c. Solution-heating at 1,200°C for 16 hours; air-cool; heat at 1,100°-1,150°C for 2-4 hours; air-cool; age at 800°C for 16 hours; air-cool.

However, for many purposes, e.g. for gas turbine nozzle guide vanes, rotor blades and integrally bladed rotors, for small gas turbines such as for automotive propulsion, auxiliary engines on aircraft or ships and for diesel engine turbo-blowers, it is extremely important that articles and parts cast from high-temperature alloys should not only have high stress-rupture strength at the aforementioned high temperatures of 927°C or 980°C, but also have a combination of high stress-rupture strength and stress-rupture ductility (as measured by the elongation at fracture) at intermediate temperatures, e.g. 816°C (1500°F).

Given the emphasis on stress-rupture strength, obtaining an improved level of ductility has not been without difficulty. For it will be appreciated that the ductility of alloys of a given base composition at a given temperature generally decreases as the stress-rupture strength is increased by minor modifications in composition. And the results in Table II of my prior Application reflect that the stronger alloys, i.e., those for which

$\frac{1}{2}$  (percent Ta) + percent Nb + percent Ti + percent Al is between 6.7 and 7.7, generally have elongations at rupture, when tested under a stress of 276 N/mm<sup>2</sup> (28 kgf/mm<sup>2</sup>) at 816°C, of less than about 4 percent. The specimens had been heat-treated by solution-

heating at 1,150°C for 4 hours, air-cooled, aged at 850°C and again air-cooled. Little improvement in ductility resulted from the interposition of an intermediate heating in between the solution-heating and aging, as in heat-treatment (b) above.

The present invention is based on the discovery that the stress-rupture ductility and the stress-rupture life at 816°C for the alloys aforescribed can be substantially improved provided there is interposed between the solution-heating and aging steps a two-stage intermediate treatment at temperatures within critical ranges.

According to the invention the alloys are given the following heat-treatment:

- i. solution-heating at 1120°-1180°C for from 2 to 16 hours (preferably at about 1150°C for about 4 hours)
- ii. heating at 970°-1030°C for from 2 to 10 hours (preferably at about 1,000°C for about 6 hours)
- iii. heating at 870°-930°C for from 8 to 48 hours (preferably at about 900°C for about 24 hours)
- iv. aging at 600°-800°C for from 8 to 48 hours (preferably at about 700°C for about 16 hours)

The alloys may be cooled at any convenient rate after each heat-treatment stage, e.g. by air-cooling (generally to room-temperature).

The improvement brought about by this four-stage heat-treatment is most surprising, particularly since I have determined that two prior art four-stage heat-treatments (there could be others) for nickel-chromium-cobalt base alloys seriously impair either the stress-rupture life or ductility at 816°C.

It is well known that if the more advanced nickel-chromium base alloys which possess the highest creep-rupture strengths attainable at a particular chromium content contain a small excess of hardening elements, sigma phase can be formed during very long time service under stress at temperatures in the range of about 800° to 870°C. This is also true for alloys of the present invention, and for such very prolonged service in this temperature range in order to eliminate the possibility of sigma phase formation (or render the amount that could be formed so small that its effect on the properties of the alloys would be negligible) (i) the value of  $\frac{1}{2}$  (percent Ta) + percent Nb + percent Ti + percent Al should not exceed 7.7 percent, (ii) the chromium content should not exceed about 23.5 percent and (iii) the W +  $\frac{1}{2}$  (percent Mo) should not be greater than about 2.5 percent.

The advantages of the heat-treatment of the invention are clearly shown by the results of tests on an alloy of the same nominal composition as Alloy No. 24 of my prior Application, namely:

- 23 percent Cr, 15 percent Co, 2 percent W, 1 percent Nb, 1.4 percent Ta, 3.5 percent Ti, 1.9 percent Al, 0.15 percent C, 0.1 percent Zr, 0.01 percent B, balance (apart from impurities) Ni.

Test-pieces machined from tapered test-bar blanks cast from a vacuum-melted heat of this alloy were given various heat-treatments and then subjected to stress-rupture tests at 816°C under a stress of 276 N/mm<sup>2</sup> and to tensile tests at 20°C. The heat-treatments and tests results are set forth in Table I.

TABLE I

| Heat Treatment                                    | Stress-rupture         |          | Tensile 20°C      |                    |
|---------------------------------------------------|------------------------|----------|-------------------|--------------------|
|                                                   | 276/816°C<br>Life, hr. | Elong. % | N/mm <sup>2</sup> | U.T.S.<br>Elong. % |
| A 4h/1150°C + 6h/1000°C<br>+24h/900°C + 16h/700°C | 1572                   | 8.8      | 941               | 3.7                |
| B 4h/1150°C + 24h/900°C<br>+16h/700°C             | 1290                   | 5.2      | 897               | 1.0                |
| C 4h/1150°C + 6h/1000°C<br>+16h/700°C             | 1327                   | 5.8      | 903               | 0.8                |
| D 4h/1150°C + 16h/850°C                           | 1358                   | 4.4      | 942               | 2.2                |
| E 4h/1163°C + 4h/1080°C<br>+24h/927°C + 16h/760°C | 1336                   | 3.4      | 1010              | 4.3                |
| F 4h/1177°C + 4h/1080°C<br>+24h/843°C + 16h/760°C | 1399                   | 4.0      | 1020              | 2.9                |
|                                                   | 907                    | 2.6      | 1030              | 1.2                |

U.T.S. = Ultimate Tensile Stress

In each case the specimens were air-cooled to room-temperature between successive stages of the heat-treatment.

Of the six heat-treatments in Table I, only Treatment A is in accordance with the invention. In each of Treatments B and C one of the two intermediate heating steps was omitted, these being examples of the three-stage heat-treatment (b) of my prior U.S. Application. Treatment D represents a prior preferred two-stage treatment. E and F are two prior art four-stage treatments described in U.K. specification No. 1,248,492.

nominal composition: 22.7 percent Cr, 19 percent Co, 2 percent W, 1 percent Nb, 1.4 percent Ta, 3.7 percent Ti, 1.9 percent Al, 0.15 percent C, 0.1 percent Zr, 0.01 percent B, Ni balance (apart from impurities). This alloy is stronger in stress-rupture than the alloy used in the tests reported in Table I, and accordingly the stress-rupture tests at 816°C were carried out under the higher stress of 310 N/mm<sup>2</sup>. The results of stress-rupture tests at 927°C under a stress of 120 N/mm<sup>2</sup> are also given.

TABLE II

| Heat Treatment                                    | Stress-rupture    |     |         | Tensile 20°C |                             |             |
|---------------------------------------------------|-------------------|-----|---------|--------------|-----------------------------|-------------|
|                                                   | N/mm <sup>2</sup> | °C  | Life h. | %<br>Elong.  | U.T.S.<br>N/mm <sup>2</sup> | %<br>Elong. |
| A 4h/1150°C + 6h/1000°C<br>+24h/900°C + 16h/700°C | 310               | 816 | 1101    | 9.4          | 950                         | 3.0         |
| D 4h/1150°C + 16h/850°C                           | 120               | 927 | 800     | 8.0          | 965                         | 3.8         |
|                                                   | 310               | 816 | 915     | 2.8          | 846                         | 0.5         |
|                                                   | 120               | 927 | 817     | 8.1          | 875                         | 0.7         |

It will be seen that Treatment A gives the best combination of rupture life and ductility and tensile ductility, the stress-rupture ductility being more than twice that given by the two-stage Treatment D with the stress-rupture life being some 20 percent greater. Treatments B and C both afford some improvement in stress-rupture ductility, but offer no significant change in stress-rupture life, and both treatments impaired tensile ductility compared with Treatment D.

The prior art four-stage Treatments E and F both seriously detracted from stress-rupture life at 816°C and tensile ductility compared with Treatment A (also D). Although Treatment E resulted in good stress-rupture ductility, this was associated with very poor stress-rupture life.

In terms of morphology, alloys contemplated herein upon being subjected to the four-stage sequence of heating have a structure characterized by the presence in the grain boundaries of small, discrete M<sub>23</sub>C<sub>6</sub>-type carbide particles without significant extra precipitation or denudation of gamma prime precipitates in adjacent areas.

Particularly good results are obtained with alloys having compositions within the following ranges: 22.2 to 22.8 percent Cr, 18.5 to 19.5 percent Co, 1.8 to 2.2 percent W, 0.9 to 1.1 percent Nb, 1.3 to 1.5 percent Ta, 3.6 to 3.8 percent Ti, 1.8 to 2.0 percent Al, 0.13 to 0.17 percent C, 0.04 to 0.12 percent Zr, 0.004 to 0.012 percent B, balance Ni. In Table II are set forth the results of tests on an alloy within this range having the

40 These data reflect that the stress-rupture life and ductility at 816°C and the tensile ductility at room-temperature are again substantially increased by Treatment A compared with Treatment D, while the stress-rupture properties at 927°C are substantially unchanged.

45 It is thought that the heat-treatment according to the invention may also advantageously be applied to the alloys in the wrought form. Moreover, it is considered that the special sequence of heating steps herein described is applicable to other nickel-chromium high temperature superalloys, particularly those hardenable by at least from 3 percent to 12 percent of titanium plus aluminium, and/or matrix hardenable by one or more of niobium, tantalum, molybdenum and tungsten, with elements such as cobalt, zirconium, boron, carbon and hafnium being optionally present.

50 I claim:

1. A heat treating process for improving properties of nickel-chromium alloys at elevated temperatures on the order of 815°C which comprises subjecting an alloy 55 consisting essentially of about 0.02 to about 0.25 carbon, about 20 to about 25 percent chromium, about 5 percent to about 25 percent cobalt, at least one metal from the group of molybdenum up to 3.5 percent and tungsten up to 5 percent in amounts such that 0.5 percent Mo plus percent W is from 0.5 to 5 percent, about 1.5 to about 5 percent titanium, about 1 to about 5 percent aluminium, the sum of the Ti and Al being from

about 4 to about 7 percent and not more than about 6 percent in tungsten free alloys, and the ratio of titanium to aluminium being about 0.75:1::4:1, about 0.5 to 3 percent tantalum, up to 3 percent niobium, about 0.005 to 1 percent zirconium, up to 2 percent hafnium, the sum of the Zr + 0.5 % Hf being from 0.01 to 1 percent about 0.001 to 0.05% boron, the balance being essentially nickel, the nickel being at least about 30 percent, to the following sequence of heat treating operations:

- a. heating at about 1,120° to about 1,180°C for about 2 to about 16 hours;
- b. heating at about 970° to about 1,030°C for about 2 to about 10 hours;
- c. heating at about 870° to 930° for about 8 to about 48 hours; and
- d. heating at about 600 to about 800°C for about 8 to about 48 hours.

2. The process in claim 1 in which heating (a) is for about 4 hours at about 1150°C.

3. The process in claim 1 in which heating (b) is for about 6 hours at about 1000°C.

4. The process in claim 1 in which heating (c) is for about 24 hours at about 900°C.

- 5. The process in claim 1 in which heating (d) is for about 16 hours at about 700°C.
- 6. The process in claim 1 in which the alloy treated contains about 0.13 to about 0.17 percent carbon, about 22.2 to about 22.8 percent chromium, about 18.5 to about 19.5 percent cobalt, about 1.8 to about 2.2 percent tungsten, about 1.3 to about 1.5 percent tantalum, about 0.9 to about 1.1 percent niobium, about 3.6 to about 3.8 percent titanium, about 1.8 to 2 percent aluminium, about 0.04 to 0.12 percent zirconium, about 0.004 to 0.012 percent boron, and the balance essentially nickel.

7. The process in claim 1 in which

- a.  $\frac{1}{2}$  percent Ta + percent Nb + percent Ti + percent Al is not greater than 7.7 percent;
- b. the chromium content does not exceed about 23.5 percent; and
- c.  $\frac{1}{2}$  percent Mo + percent W is not greater than about 2.5 percent.

8. The alloy produced by the process of claim 1 having a structure characterized by the presence in the grain boundaries of small, discrete  $M_{23}C_6$ -type carbide particles without significant extra precipitation of gamma prime precipitate in adjacent areas.

\* \* \* \* \*

30

35

40

45

50

55

60

65